

[54] ACID RESISTANT ALLOYS

[75] Inventor: **Maharaj K. Koul**, Lewiston, N.Y.

[73] Assignee: **Union Carbide Corporation**, New York, N.Y.

[22] Filed: **Jan. 15, 1973**

[21] Appl. No.: **323,787**

**Related U.S. Application Data**

[63] Continuation of Ser. No. 80,812, Oct. 14, 1970, abandoned.

[52] U.S. Cl. .... **75/174, 75/175.5**

[51] Int. Cl. .... **C22c 27/00**

[58] Field of Search. .... **75/174, 175.5, 134 N**

[56] **References Cited**

UNITED STATES PATENTS

2,822,268 2/1958 Hix ..... 75/174

3,317,314 5/1967 Wlodek et al. .... 75/174

**FOREIGN PATENTS OR APPLICATIONS**

803,855 11/1958 Great Britain

889,099 2/1962 Great Britain

925,107 5/1963 Great Britain

*Primary Examiner*—Hyland Bizot

*Assistant Examiner*—E. L. Weise

*Attorney, Agent, or Firm*—Frederick J. McCarthy, Jr.

[57] **ABSTRACT**

An acid resisting alloy consisting essentially of about 10 to 50 percent titanium, 50 to 85 percent columbium, 5 to 10 percent tungsten, and 0.5 to 3 percent zirconium.

**1 Claim, No Drawings**

## ACID RESISTANT ALLOYS

This is a continuation, of application Ser. No. 080,812 filed Oct. 14, 1970 now abandoned.

This invention relates to acid resistant alloys. More particularly this invention relates to titanium containing alloys which are resistant to oxidizing as well as reducing media. While alloys are known which are resistant to either oxidizing acids such as nitric acid or reducing acids such as hydrochloric acid at present there is no known material which is resistant to hot concentrated reducing and oxidizing acids. Such an alloy would be highly useful for applications in the chemical industry such as autoclaves, seals and acid tanks.

It is therefore an object of the present invention to provide an alloy which is highly resistant to both oxidizing and reducing media.

Other objects will be apparent from the following description and claims.

An alloy in accordance with the present invention consists essentially of from about 10 to 50 percent titanium, 50 to 85 percent columbium, 5 to 10 percent tungsten and 0.5 to 3 percent zirconium. A preferred alloy in accordance with the present invention is one containing about 26 percent titanium, 65 percent columbium, 7.5 percent tungsten and 1.5 percent zirconium.

Alloys in accordance with the present invention are readily melted by vacuum arc melting techniques and can be readily fabricated into industrially useful forms such as sheet, plate and the like.

The following examples will further illustrate the present invention.

## EXAMPLE I

Alloy test specimens having a composition of 26% Ti, 65 percent Cb, 7.5 percent W and 1.5 percent Zr in the form of 1 inch  $\times$  1 inch  $\times$  0.03 inch sheet samples were tested in 20 percent HCl at 70°C, boiling H<sub>2</sub>SO<sub>4</sub> (40 percent), and boiling 65 percent nitric acid. Similarly sized test specimens of an alloy having a composition of Ti, 0.2 percent Pd were also tested in the same manner. The results of the tests are shown in Table I.

Table I

45

| Alloy Composition wt-%                | Test Media                                                                                                | Corrosion Rate in/year |
|---------------------------------------|-----------------------------------------------------------------------------------------------------------|------------------------|
| 26% Ti, 65% Cb,<br>7.5% W and 1.5% Zr | 65% HNO <sub>3</sub><br>(Boiling)<br>20% HCl<br>(70°C)<br>40% H <sub>2</sub> SO <sub>4</sub><br>(Boiling) | Nil<br>.001<br>.02     |
| Ti-0.2% Pd.                           | 65% HNO <sub>3</sub><br>(Boiling)<br>20% HCl<br>(70°C)<br>40% H <sub>2</sub> SO <sub>4</sub><br>(Boiling) | .025<br>.010<br>2.2    |
|                                       |                                                                                                           |                        |

## EXAMPLE II

Alloy test specimens having a composition of 26 percent Ti, 65 percent Cb, 7.5 percent W and 1.5 percent Zr in the form of 1 inch  $\times$  1 inch  $\times$  0.03 inch were tested by exposure to the "off-gas" condensate from a vanadium salt roast process at a temperature of 90°-100°C. The "off-gas" condensate contained approximately 17 percent HCl and 1.5 percent HF.

Test specimens in the form of 1 inch  $\times$  1 inch  $\times$  0.03 inch sheet samples of alloys having compositions of Ti - 0.2 percent Pd and Ti - 26 percent Mo were also tested in the "off-gas" condensate. The results are shown in Table II.

Table II

| Alloy Composition                  | Test Media                       | Corrosion Rate |
|------------------------------------|----------------------------------|----------------|
| 26% Ti, 65% Cb, 7.5% W and 1.5% Zr | "Off-Gas" Condensate at 90-100°C | 0.004 in/yr    |
| Ti - 0.2% Pd                       | do.                              | 27.6 in/yr     |
| Ti - 26% Mo                        | do.                              | 0.81 in/yr     |

I claim:

1. An alloy of titanium, columbium, tungsten and zirconium resistant to hot oxidizing and reducing acids consisting essentially of about 26 percent titanium, 65 percent columbium, 7.5 percent tungsten, and 1.5 percent zirconium.

\* \* \* \* \*

50

55

60

65